

June 11, 1929.

C. J. WRIGHT

1,716,572

PROCESS AND APPARATUS FOR BURNING LIME

Filed Aug. 15, 1923

3 Sheets-Sheet 1



June 11, 1929.

C. J. WRIGHT

1,716,572

PROCESS AND APPARATUS FOR BURNING LIME

Filed Aug. 15, 1923.

3 Sheets-Sheet 2



June 11, 1929.

C. J. WRIGHT

1,716,572

PROCESS AND APPARATUS FOR BURNING LIME

Filed Aug. 15, 1923

3 Sheets-Sheet 3

*Fig. 3*



*Fig. 4*



Inventor

CARL J. WRIGHT

By his Attorney

Edmund G. Borden

## UNITED STATES PATENT OFFICE.

CARL J. WRIGHT, OF WEST NEW BRIGHTON, NEW YORK, ASSIGNEE, BY MESNE ASSIGNMENTS, TO COMBUSTION UTILITIES CORPORATION, OF NEW YORK, N. Y., A CORPORATION OF MAINE.

## PROCESS AND APPARATUS FOR BURNING LIME.

Application filed August 15, 1923. Serial No. 657,492.

This invention relates to the manufacture of lime and carbonic acid gas from carbonates in a continuous manner.

A large part of the lime made in this country is calcined in a kiln either in direct contact with the fuel or with the fuel gases, so that the ultimate products are more or less impure. In such a process the gaseous products of combustion of the fuel such as nitrogen of the air used for combustion, sulphur dioxide and ammonia become mixed with the carbonic acid gas, giving a gaseous product with a low carbonic acid content, which is not efficient for use in soda ash manufacture, and is too impure for other purposes. In addition to giving impure carbonic acid gas, this method of burning lime is expensive and inefficient, and is difficult to control, often resulting in underburning or overburning a part of the lime. Moreover, the solid and liquid products of decomposition of the fuel, such as ash, tar and clinkers are withdrawn in considerable amount mixed with the lime, resulting in an unclean lime with poor slackening qualities. Various attempts have been made to overcome these difficulties by employing other heating means, in particular currents of superheated air or superheated steam, but it is not known that any of these attempts have resulted in a process which could be adopted in general commercial practice.

The primary object of the present invention is to provide a process for burning lime by which lime may be efficiently and economically produced and comparatively pure carbonic acid gas may be obtained while burning lime.

Another object of the present invention is to provide a process for burning lime by which a minimum amount of heat is lost due to the removal of highly heated products from the apparatus in which the process is carried out.

Another object of the present invention is to provide a process for burning lime by which the temperature will be accurately controlled so that the lime will not be under or over burned.

Another object of the present invention is to provide a commercially practicable process for burning lime by which the decomposition

temperature of the lime is obtained solely by heat transfer from a chemically inert gaseous mixture.

A further object of the invention is to provide an apparatus in which lime may be efficiently burned and the above process carried out.

With these and other objects in view the invention consists in the improved process and apparatus for burning lime hereinafter described and claimed.

The various features of the invention are illustrated in the accompanying drawings, in which

Fig. 1 is a more or less diagrammatical view in side elevation with parts in section of a lime burning kiln and the auxiliary gas treating apparatus embodying the preferred form of the invention.

Fig. 2 is a view in plan partly in section of the apparatus shown in Fig. 1.

Fig. 3 is an enlarged horizontal cross sectional view of the lower portion of the kiln showing in plan the mechanism for supporting a charge column of limestone in the kiln and for removing charge material from the foot of the column.

Fig. 4 is an enlarged view in vertical section of the charge supporting and discharge mechanism shown in plan in Fig. 3, taken on the line 4-4 of Fig. 3.

The process and apparatus of the present invention is so designed that lime may be economically and continuously burned and substantially pure lime and carbonic acid gas may be obtained. By the use of an improved apparatus any gaseous medium preferred may be superheated to the temperature desired for carrying on a chemical reaction. According to the preferred form of this invention a mixture of carbonic acid gas and steam is superheated to a temperature of about 1900° F. to 2000° F., and then passed through a column of limestone in a kiln for burning it. The action of the inert gas on the limestone may be accurately controlled as to temperature, so that the lime will not be under or over burned, and the resulting gaseous mixture composed of carbon dioxide and steam can be run

through a condenser to remove the steam, leaving substantially pure carbon dioxide gas. The gaseous mixture is superheated by

use of the commonly used regenerators, recuperators or similar heat exchanging apparatus. A cheap grade of fuel is used for heating preheaters and regenerators and by 5 utilizing efficient types of preheaters and heat exchangers, and a special type of kiln, the present process and apparatus enables the production of lime and carbonic acid gas at a considerably lower cost than has heretofore 10 been realized in commercial practice.

To carry out the improved process in the apparatus illustrated in the drawings, limestone is passed in a column downwardly through a shaft kiln 10, Fig. 1. The limestone 15 is dropped from a bin 12 into a charging hopper 14 located at the top of the kiln, by opening a gate 16 on the bottom of the bin. The gate 16 is then closed and a gate 18 at the bottom of the charging hopper is opened, per- 20 mitting the limestone in the charging hopper to flow into the top of the kiln. The charging operation is an intermittent one, and the gates 16 and 18 are so operated that while one is open the other will always be closed, 25 in order to prevent the escape of gases from the kiln into the bin. The limestone is sup- ported in the furnace in a vertical column, and is continuously advanced downwardly through the column. In its passage through 30 the furnace the column of lime is passed through three distinct zones, namely, a heating zone 20, in the upper part of the shaft, a hot mid zone 22, and a lime cooling zone 24 in the lower part of the shaft. The limestone 35 is decomposed in the mid zone 22 of the kiln, at a temperature of from 1400° to 2000° F., into lime and carbonic acid gas, according to the following reaction:



The gate 26 is shown as a revolving truncated hollow cone with a segment of its wall cut out, forming a slot. This cone is adjustable in order that it will always take up wear 45 and provide a gas tight seal during the periods of discharge.

The circuit of gas and steam which is used as the sole medium to maintain the high temperatures in the mid zone 22 of the shaft, is 50 heated by being passed through a preheater in contact with a body of highly heated refractory material. This refractory material has been previously heated by the heat of combustion of producer gases which have been 55 generated in some form of stoker.

The stoker indicated as 28 in Fig. 2 may be an ordinary coal furnace, a gas producer, a gas burner or an oil burner. In this stoker the cheapest type of fuel can be burned, and 60 the products of combustion are sent through hot conduits 30 or 32, to one of a pair of regenerators or preheaters 34 or 36, as shown. The circulation of the hot gases is controlled by hot valves 38 and 40 which are especially 65 designed to withstand high temperatures,

and preferably, arrangement is made so that the pressure on the opposite sides of the valves is substantially the same, so that there is a minimum leakage. When one regenerator is being heated by the hot gases, the other re- 70 generator which has previously been heated is used for preheating carbonic acid gas and steam. The hot furnace gases after passing through either of the regenerators are drawn through conduits 42 or 44, 75 provided with hot valves 46 or 48, into feed water heaters 50 and 52, and from the feed water heaters they are exhausted to the atmosphere through stack pipes 54, 56 or 58, 60, and exhausters 62 or 64. The feed water 80 heaters have water pipe connections 66 and 68 with a steam boiler 70, and a part of the hot gases from the stoker are drawn through a conduit 72 to be utilized in generating steam in the boiler, at substantially 212° F. and 85 atmospheric pressure. The only pressure built up in the boiler is that required for positively controlling the circulation of steam.

Steam from the boiler is admitted into the 90 lower end of the kiln by means of pipes 74 connected to a horizontal coil 76 placed a short distance above the discharge gate, said coil being perforated in such a way that the steam will be evenly distributed throughout 95 the body of lime in the lower part of the kiln.

To support the column of lime and to insure an equalized downward movement of the charge throughout the kiln, as well as to aid in evenly distributing steam throughout the 100 body of the charge, a grate is set in the lower part of the shaft just above the steam coil 76. In its preferred form this grate may consist of a series of hoppers 78, that is six peripheral hoppers and a central hopper, formed 105 respectively by the opposed sloping sides of six uniformly spaced and peripherally disposed, stationary tent shaped supporting members 79 and a centrally disposed ring shaped member 81 of conical cross section 110 connected therewith, with discharge openings 80 in the bottom of each peripheral hopper through which the lime passes from the bottom of the column onto a series of movable platforms 82. The platforms 82 are 115 given a reciprocating motion by means of water operated engines 84, to discharge the lime from the platforms into a hopper 86, forming the bottom of the shell. A more complete description of this discharge mech- 120

anism will be found in the British patent to Henry O. Loebell, No. 216,488, May 23, 1923. The amount of steam admitted into the bottom of the charge through the perforated coil 76 is controlled so as to cool the lime at the discharge gate to a comparatively low temperature, that is, to as low a temperature as is consistent with the production of quick lime as distinguished from slack lime at the base of the column, or in other words to a 130

temperature above the dissociation temperature of calcium hydrate. In burning limestone to recover lime and carbonic acid gas, the reaction which takes place is reversible 5 in cases where an excess of carbonic acid gas may come in contact with the lime. The introduction of steam into the bottom of the charge drives out any carbonic acid gas which might be carried down with the lime, prevents any reversal of the primary reaction 10 and insures the complete burning of the lime. As the steam rises toward the high temperature zone it takes up heat from the descending body of burnt lime and itself becomes superheated to a temperature corresponding 15 to the high temperature zone of the furnace as it reaches that zone.

The heat transferring medium which is used in the present process for heating the 20 mid zone of the descending body of limestone to a temperature such that complete decomposition takes place, consists of inert gases, and is preferably composed of about 70%  $\text{CO}_2$  and 30% steam by weight. The mixture 25 of carbonic acid gas and steam is forced by a blower through the hot brick work 88 of one of the pair of regenerators or preheaters shown, while the other regenerator is being heated by recovering the heat of combustion 30 of furnace gas therein. When one regenerator has been cooled to the minimum working temperature which is desirable, by passing carbonic acid gas and steam through it, the circulation of the steam and  $\text{CO}_2$  mixture is 35 stopped and then started in the other regenerator, which was being heated during the time when the first regenerator was used for heating the mixture of steam and  $\text{CO}_2$ . In passing through the regenerator the gas mixture 40 becomes superheated to a temperature of about 2000° F. and it then flows through a blast neck 90 or 92 and hot valves 94 or 96 into a passage 98 surrounding the fuel column, by means of which it is evenly distributed 45 throughout the cross-section of the column. Here the mixture of blast gases is joined by the steam which was introduced at the bottom of the column of lime, and by the carbonic acid gas produced in the decomposition 50 of the limestone. As this body of mixed gases ascends toward the top of the kiln it is cooled by a heat transfer with the body of descending limestone in the heating zone 20 so that the limestone is gradually 55 heated as it approaches the high temperature zone 22 of the kiln, and the mixed gases as they approach an offtake pipe 100 at the top of the kiln are gradually cooled to a temperature of about 500° F. The speed with which 60 the body of limestone traverses the length of the kiln, and with which the mixed gases are drawn through the kiln, is controlled by the speed of the reciprocating tables 82 and an exhauster 102, respectively, so as to give a 65 good heat recovery and a resultant good heat

balance. After passing through the offtake the mixture of gases is divided at the T 104, a part being recirculated through the blower 102 and pipes 106 or 108 through the regenerators and kiln to maintain the high temperature in the mid portion of the body of lime, while the remainder of the gas mixture is run through a tubular condenser 110, in which the steam is condensed and from which the practically pure carbonic acid gas may be passed 70 through a fan 116 and discharge pipe 117 to soda ash absorption towers or to other use in the arts. The condensed steam and the water from the tubular condenser may be led to the feed water heaters by pipes 112 and 80 114, and from there to the boiler, if desired. The amount of gas passing the offtake which is recirculated, and the amount which is withdrawn through the condenser, is governed by the speed of the exhauster 102, and 85 the speed of the fan 116 in the condenser circuit.

The shaft furnace 10 is arranged to support the fuel in a vertical column in such a manner that the limestone may be continuously advanced through the furnace while it is being continuously calcined. The furnace 10 consists of a cylindrical gas-tight metal shell 118, provided with a refractory lining 120 and having a top cover consisting of the charging 90 hopper 14 and the bin 12, with the intermittently operating charging valves 16 and 18, and a lime discharging hopper 86 at its lower end in which the discharge gate 26 is located. The refractory lining 120 is preferably positioned in all the inner surface of the shell which comes into contact with the heated limestone. The shell and lining are both so constructed as to gradually increase 95 the cross-sectional area of the column of lime- stone as it advances to the mid zone of the furnace, in order that it may expand into a larger space to be in an open condition to assist the cross blast in penetrating through the column. The refractory lining is constructed so as to 100 form a flat fire arch 122 immediately above the blast necks 90 and 92 thus forming the passage 98 between the descending body of the charge and the lining immediately beneath the flat arches around the whole circumference of the shaft, through which the hot gases will distribute themselves equally throughout the central section of the descending charge. These flat arches confine the cross 105 blast of superheated gases to the zone 22 and prevent a direct application of the hot blast gases into the heating zone 20. The shell and lining below the expanded hot mid zone of the furnace is so built as to gradually contract 110 the cross sectional area of the column of lime as it descends from the hot mid zone toward the discharge, so that the calcined lime, which has lost in volume during the burning process, is compressed gradually as it cools, by the 115 weight of the descending column, and this 120

compression of the burnt lime assists the cooling and cleansing action of the steam rising from the coil 76.

The regenerators or preheaters 34 and 36 5 for preheating the inert blast gases and for absorbing the heat of the stoker gases preferably consist of cylindrical gas-tight shells which have refractory linings 124 covering their inner surface. The heat recuperation 10 of the gases in the regenerators is effected mainly by means of a series of checker bricks 88 which are supported on grates positioned near the bottom of the shells and extend to the level of the flues 30, 32, 90 and 92. Hot 15 valves are positioned in the stoker conduit, the blast neck, the gas circuit line from the blower, and the combustion gas conduit between the regenerator and feed water heater, so that the regenerator may be cut off from 20 the gas circuit while it is being heated by the combustion gases from the stoker, and then may be cut off from the stoker and feed water preheater while heating the circuit of blast gases. The construction 25 of these hot valves is clearly explained in the British patent to Loebell No. 216,488. The valve essentially consists in a block of refractory material, which is connected to a head, and is moved through slots in the conduit in which the valve is located, by hydraulic power.

In case no supply of carbonic acid gas or of 30 mixed carbonic acid gas and steam is readily available at the time the present lime burning process is first put into operation after a shutdown, the heat required for putting the process into the continuous normal operation above described is supplied in the following manner: After introducing a charge of limestone into the kiln a high degree of preheat 35 is first imparted to the refractory linings of preheaters 34 and 35, preferably by the combustion of gaseous fuel from stoker 28 in heat transferring relationship therewith, and steam is then conducted from boiler 70 40 through branch pipe connections 126 and conduits 108 preferably into the base of both preheaters. In passing through the heated linings of the preheaters a high degree of 45 superheat, about 1900° to 2000° F. is imparted to the steam and this superheated steam is then sent through the charge of limestone to raise the temperature of the charge to that 50 point at which decomposition into calcium oxide and carbonic acid gas begins in the blast zone. After thus initiating the lime burning operation this initial supply of superheated steam is preferably cut-off by 55 closing valves 128 in the pipes 126 and thereafter the heat supply for maintaining the lime burning operation is carried to the charge by the circuit of mixed steam and carbonic acid gas withdrawn from the top of the kiln, as already described.

60 From the foregoing description it is evi-

dent that a very efficient recovery of heat is obtained from the combustion of the cheapest type of fuel in the stoker, and also from the solid and gaseous products of the decomposition of limestone in the furnace. This efficient heat recovery and the fact that a 70 cheap fuel may be utilized, cuts the cost of fuel to less than a half of that necessary in present day lime burning operations. At the same time practically pure products are produced; and the control of the operation is so 75 closely governed as to insure that the lime will always be burned to just the degree desired.

By using a mixture of steam with carbonic acid gas, or other chemically inert gases such 80 as air or nitrogen the tension of the expelled carbonic acid gases is reduced, due to partial pressures, and this fact permits the liberation of the carbonic acid gas at somewhat 85 lower temperatures and in a shorter period of time than is obtained by using a single gas as heating medium.

The preferred form of the invention having been thus described what is claimed as 90 new is:

1. A process of burning limestone comprising, continuously passing limestone downwardly in a column through a shaft kiln, effecting continuous thermal decomposition of the limestone in the mid-portion of the column by contacting it with a stream of preheated inert gas, cooling the lime product of said decomposition in the lower portion of the column by contacting it with a counter-flow stream of saturated steam, and 100 continuously withdrawing cool lime from the foot of said column and a cool mixture of steam and carbon dioxide from the top of 105 said column.

2. A process of burning limestone comprising, continuously passing limestone downwardly in a column through a shaft kiln, effecting continuous thermal decomposition of the limestone in the mid-portion of the column by contacting it with a stream of preheated inert gas, cooling the lime product of said decomposition in the lower portion of the column by contacting it with a counter-flow stream of saturated steam, continuously withdrawing lime from the foot of said column and a cool mixture of steam and carbon dioxide formed from the top of said column, and controlling the temperature and volume of said inert gas stream and the volume of said saturated steam cooling medium to prevent under or over burning of lime in said decomposition zone. 110

3. A process of burning limestone comprising, continuously advancing limestone downwardly in a column through a shaft kiln, effecting continuous thermal decomposition of said limestone by contacting it with a superheated mixture of steam and carbon dioxide introduced circumferentially 115 120 125 130

into the mid-portion of said column and passed upwardly therethrough, cooling the lime product of said decomposition by contacting it with steam introduced at the base 5 of said column and passed upwardly therethrough, and controlling the volume of saturated steam thus introduced to maintain the temperature of the lime at the foot of said column only slightly above the dissociation 10 temperature of calcium hydrate.

4. A process of burning limestone comprising, continuously advancing limestone downwardly in a column through a shaft kiln, effecting continuous thermal decomposition 15 of the limestone in the mid-portion of said column by direct heat transfer with a superheated mixture of steam and carbon dioxide, regenerating a substantial part of the sensible heat of the lime formed by heat 20 transfer with saturated steam introduced at the foot of the column and passed upwardly therethrough, regenerating a substantial part of the sensible heat of the carbon dioxide formed by contacting it with the limestone in the upper part of the column, and withdrawing lime from the foot of the column and a carbon dioxide-steam mixture 25 from the top of the column.

5. A process of burning limestone comprising, continuously advancing limestone downwardly in a column through a shaft kiln, effecting continuous thermal decomposition 30 of the limestone in the mid-portion of said column by direct heat transfer with a superheated mixture of steam and carbon dioxide, regenerating a substantial part of the sensible heat of the lime formed by heat transfer with saturated steam introduced at the foot of the column and passed upwardly there- 35 through, regenerating a substantial part of the sensible heat of the carbon dioxide formed by contacting it with the limestone in the upper part of the column, withdrawing cooled lime from the foot of the column and a cool 40 carbon dioxide-steam mixture from the top of the column, and superheating part of the carbon dioxide-steam mixture thus withdrawn and reintroducing it into the mid-portion of said column.

50 6. A process of burning limestone comprising, continuously advancing limestone downwardly in a column through a shaft kiln, effecting continuous thermal decomposition of the limestone in the mid-portion of said column by direct heat transfer with a superheated mixture of steam and carbon dioxide passed upwardly therethrough, regenerating a substantial part of the sensible heat of the lime formed by heat transfer with steam introduced at the foot of the column and passed upwardly therethrough, regenerating a substantial part of the sensible heat of the carbon dioxide formed by contacting it with the limestone in the upper part of the column, continuously withdrawing cool lime at a con- 65

trolled rate from the foot of the column and a cool carbon dioxide-steam mixture from the top of the column, and continuously superheating a part of the carbon dioxide-steam mixture thus withdrawn and recycling it 70 through the upper half only of said column.

7. A process of burning limestone comprising, continuously passing limestone downwardly in a column through a shaft kiln, effecting continuous thermal decomposition of 75 the limestone in the mid-portion of the column by contacting it with a counter-flow mixture of super-heated steam and carbon dioxide, preheating the limestone in the upper part of the column prior to such decomposition by contacting it with the carbon dioxide product of said decomposition, superheating steam used in effecting such decomposition by contacting it with the lime product of said decomposition in the lower 80 part of the column, continuously withdrawing cool lime at a controlled rate from the foot of the column and a cool steam-carbon dioxide mixture from the top of the column, superheating a part of the steam-carbon dioxide mixture thus withdrawn and recycling it through the upper half of the column, and supplementing the volume of said recycled mixture with the steam superheated 85 in the lower part of the column and with the 90 carbon dioxide product of said decomposition.

8. A process of burning limestone comprising, continuously passing limestone downwardly in a column through a shaft kiln, effecting continuous thermal decomposition of the limestone in the mid-portion of the column by contacting it with a counterflow mixture of superheated steam and carbon dioxide, preheating the limestone in the upper 100 part of the column prior to such decomposition by contacting it with the carbon dioxide product of said decomposition, superheating steam used in effecting such decomposition by contacting it with the lime product of 105 said decomposition in the lower part of the column, continuously withdrawing lime at a controlled rate from the foot of the column and a steam-carbon dioxide mixture from the top of the column, superheating part of the steam-carbon dioxide mixture 110 thus withdrawn and recycling it through the upper half of the column, supplementing the volume of said recycled mixture with the steam superheated in the lower 115 part of the column and with the carbon dioxide product of said decomposition, and separating steam from the part of the carbon dioxide-steam mixture not thus recycled and collecting the carbon dioxide resulting from 120 said separation.

9. A process of burning limestone comprising, continuously passing limestone downwardly in a column through a shaft kiln, effecting continuous thermal decomposition of 125

the limestone in the mid-portion of the column by contacting it with a counter-flow mixture of superheated steam and carbon dioxide, preheating the limestone in the upper 5 part of the column prior to such decomposition by contacting it with a counter-current stream of carbon dioxide product of said decomposition, superheating steam used in effecting such decomposition by contacting it 10 with the lime product of said decomposition in the lower part of the column, continuously withdrawing lime at a controlled rate from the foot of the column and a steam-carbon dioxide mixture from the top of the column, 15 superheating part of the steam-carbon dioxide mixture thus withdrawn and recycling it through the upper half of the column, supplementing the volume of said recycled mixture with the steam superheated in the lower 20 part of the column and with the carbon dioxide product of said decomposition, and controlling the volume of saturated steam introduced into the foot of the column to maintain the composition of the steam-carbon dioxide 25 mixture removed from the top of the column substantially constant.

10. A process of burning limestone comprising, continuously advancing limestone downwardly in a column through a shaft 30 kiln, heating the limestone in the mid-portion of the column to a temperature sufficiently high to decompose it by contacting it with a superheated mixture of steam and carbon dioxide gas, cooling the lime formed as it advances toward the foot of the column by contacting with steam, gradually expanding the limestone as it advances toward the mid-portion of the column, gradually compressing the lime formed as it advances toward the 40 foot of the column, and withdrawing comparatively cool lime from the foot of the column and comparatively cool carbonic acid gas and steam from the top of the column.

11. A process of burning limestone comprising, continuously advancing limestone downwardly in a column through a shaft kiln, heating the limestone in the mid-portion of the column to a temperature sufficiently high to decompose it by contacting it with a 45 superheated mixture of steam and carbon dioxide gas, cooling the lime formed as it advances toward the foot of the column by contacting with steam, gradually expanding the limestone as it advances toward the mid-portion 50 of the column, gradually compressing the lime formed as it advances toward the foot of the column, withdrawing comparatively cool lime from the foot of the column and comparatively cool carbonic acid gas and 55 steam from the top of the column, and controlling the volume of steam introduced at the foot of the column and the temperature and volume of said superheated carbon dioxide-steam mixture to prevent under- or over- 60 burning of the lime and to maintain the com- 65

position of the carbon dioxide-steam mixture removed from the top of the column substantially constant.

12. A process of burning limestone comprising, continuously advancing limestone 70 downwardly in a column through a shaft kiln, superheating a mixture of carbonic acid gas and steam, decomposing said limestone by introducing said superheated carbonic acid gas-steam mixture into the mid-portion of the column and passing it upwardly in contact with the limestone in the upper half of the column, supplementing the heating effect of said superheated carbonic acid-steam mixture with an additional supply of 80 superheated steam developed in the lower portion of the column at the expense of heat regenerated from the lime product of said decomposition, withdrawing lime from the foot of said column and a carbonic acid gas-steam mixture from the top of said column, maintaining the composition of the carbonic acid gas-steam mixture thus withdrawn substantially constant at about 30% steam and 70% carbonic acid gas by weight, and superheating and recycling a portion of said carbonic acid gas-steam mixture through the upper half of said limestone column. 85

13. A process of burning limestone comprising, continuously passing limestone 90 downwardly in a column through a shaft kiln, effecting continuous thermal decomposition of the limestone in the mid-portion of the column by contacting it with a superheated mixture of steam and carbonic acid gas, continuously circulating superheated steam and carbonic acid gas through the upper half of said column, regenerating the sensible heat of the carbonic acid gas formed by heat transfer with limestone in the upper portion of the column, regenerating the sensible heat of the burnt lime by heat transfer with steam in the lower portion of the column, returning the heat thus regenerated to the mid-portion of the column in the form of preheated limestone and superheated steam, respectively, and continuously withdrawing the lime from the foot of the column and a carbonic acid gas-steam mixture from the top of the column. 100

14. A process for burning limestone comprising passing a column of limestone through a shaft kiln, decomposing said limestone by introducing a superheated gaseous mixture comprising carbonic acid gas and steam into the mid portion of said column, introducing saturated steam into the bottom of the column in an amount such that the gas mixture leaving the top of the column will contain approximately 30% steam and 70% CO<sub>2</sub> by weight, superheating a part of the gas mixture drawn from the top of the shaft by passing it through a hot preheater, and returning said superheated gas mixture to the shaft. 120

15. A process for burning limestone com- 125

prising passing a column of limestone through a shaft kiln, decomposing the limestone into lime and carbonic acid gas by direct contact with a counter-current circuit of superheated steam and carbonic acid gas during its passage through the kiln, withdrawing carbonic acid gas and steam from the top of the column, and regulating the rate at which limestone is passed through the kiln and the volume and composition of the gas circuit passed countercurrently therethrough to maintain the temperature of the mixture of carbonic acid gas and steam leaving the top of the column in the neighborhood of 500° F.

16. In lime burning apparatus, an upright shaft kiln, a gas sealed charging device at the top of the shaft, a gas sealed discharging device at the foot of the shaft, means mounted in the lower portion of the shaft for supporting a charge column therein, said means having combined therewith mechanism for removing charge material at a controlled rate from the foot of the column, a gas offtake at the top of the shaft, a gas intake in the mid-portion of the shaft, means for introducing steam at a controlled rate into the lower portion of the shaft, a gas preheater, a blower, a gas connection between said offtake and the intake side of said blower, a valved connection between the discharge side of said blower and said preheater, and a valved gas connection between said preheater and the gas intake in said shaft.

17. An apparatus for burning lime comprising an upright shaft, a discharging device at the top of the shaft, a discharging device at the bottom of the shaft, a circumferential enlargement and a gas inlet in the mid portion of the shaft, a gas outlet in the top portion of the shaft, a preheater, means for circulating gas from the gas outlet through the preheater and gas inlet back into the mid-portion of the shaft, and means for introducing a heating gas into the preheater.

18. An apparatus for burning lime comprising a shaft kiln, a charging device for charging limestone into the top of the shaft, a discharging device for discharging lime from the bottom of the shaft, means for controlling the movement of lime through the shaft, a gas offtake at the top of the shaft, a pair of preheaters connected to gas inlets in the mid portion of the shaft, means for heating said preheaters, a blower, a gas connection between the intake of said blower and said gas offtake, separate gas connections between the discharge of said blower and each of said preheaters, and valves in said blower-preheater gas connections.

19. An apparatus for burning lime comprising an upright shaft-kiln, means for introducing limestone into the upper portion of the shaft, means for removing lime from the bottom of the shaft, a gas offtake connected with the top of the shaft, a pair of

gas inlets connected with the central portion of the shaft, a preheater connected with each inlet and with the gas offtake, means to introduce a heating gas into the preheaters, means for introducing a mixture of inert gases into the preheaters to be heated, means for circulating inert gases from preheaters through the gas inlets and upper portion of the shaft, and means for cutting of one preheater from the shaft when the other preheater is used to superheat the mixture of gases being introduced into the shaft.

20. An apparatus for burning lime comprising an upright shaft kiln, means for introducing limestone into the upper portion of the shaft, means for removing lime from the bottom of the shaft, a gas offtake at the top of the shaft, a pair of preheaters connected to gas inlets in the mid portion of the shaft, means for circulating gas from the offtake through the preheaters, gas inlets and upper portion of the shaft, a boiler for generating steam, feed water heaters, means for supplying heat to the preheaters, boiler and feed water heaters, water connections between said boiler and heaters, and steam connections between said boiler and shaft kiln.

21. An apparatus for burning lime comprising an upright shaft kiln, means for charging limestone into the top of the shaft, means for discharging lime from the bottom of the shaft, means connected to a gas inlet in the mid-portion of the shaft for preheating a mixture of gases before its introduction into the mid portion of the shaft, means for introducing steam into the bottom of the shaft, a gas offtake at the top of the shaft, a blower, a condenser, and connections for recirculating a portion of the gases drawn from the top of the shaft through the blower and back through the preheating means into the mid portion of the shaft, and connections for withdrawing the remainder of the gases drawn from the top of the shaft through the blower and condenser.

22. An apparatus for burning lime comprising an upright shaft, a charging device at the top of the shaft, a gas offtake at the top of the shaft, preheaters connected to the gas offtake and to blast inlets in the central portion of the shaft, a steam distributing coil in the bottom of the shaft, a steam boiler, a condenser connected with the gas offtake, feed water heaters connected to the preheaters, and connections for leading water from the condenser through the feed water heaters to the boiler, and connections for leading steam from the boiler to the coil in the bottom of the shaft and to the preheaters.

23. In an apparatus for burning lime, an upright shaft kiln, a charging device at the top of the shaft, a discharging device at the foot of the shaft, means mounted in the lower portion of the shaft for supporting a charge

column in the shaft and for controlling the movement of charge material through the shaft, a gas offtake at the top of the shaft, means for introducing hot gas into the mid-portion of the shaft, means for introducing steam at a controlled rate into the lower portion of the shaft, and means for circulating gas removed through said offtake back

through said hot gas introducing means and the upper part of the shaft, said shaft having its largest interior cross sectional dimensions at its midzone and gradually decreased cross sectional dimensions toward its top and bottom extremities.

In testimony whereof I affix my signature.  
**CARL J. WRIGHT.**